

Patented Dec. 1, 1936

2,062,666

## UNITED STATES PATENT OFFICE

2,062,666

## PELLETED BLASTING POWDER

William E. Kirst, Woodbury, N. J., assignor to  
 E. I. du Pont de Nemours & Company, Wil-  
 mington, Del., a corporation of Delaware

No Drawing. Application April 27, 1933,  
 Serial No. 668,221

10 Claims. (Cl. 52-17)

This invention relates to improved blasting powder compositions and more particularly to such deflagrating compositions in the form of blocks or sticks, containing ammonium nitrate 5 as an ingredient.

Black powder has long been known and used as a commercial explosive of relatively low velocity. The composition of this explosive has, in general, varied little over a period of many years, 10 a representative composition comprising, for example, 72% sodium nitrate, 10% sulfur, and 18% charcoal. While these ingredients have varied somewhat in amounts, the powder has retained, in general, the same approximate composition.

15 Black powder was for many years used in the form of grains of varying size. These grains were given a smooth polished surface coating by the operation known as "glazing".

More recently, however, black blasting powder 20 has been put up and used in the form of packaged sticks similar to dynamite. These sticks or blocks are produced by several well-known methods. For example, the so-called pelleted powder has largely replaced the granular powder recently for 25 blasting work. Pelleted black blasting powder is made on a press in the form of cylindrical blocks customarily, about 2" in length and of any desired diameter, for example, up to approximately 2". Ordinarily, these pellets have a hole 30 running longitudinally through their centers, this hole being about  $\frac{1}{4}$ " in diameter. It is the practice to wrap together several of these pellets, placed end to end, in a roll of paper to make a packaged explosive similar in form to a stick of dynamite.

Another method of producing black blasting powder in stick form is to pack the loose powder 35 in a formed cylindrical paper shell. Preferably, the wet powder containing, for example 4% to 40 8% of water is packed lightly in the shell. The powder is then dried in the shell. When dry, the shells are completely closed and, if desired, protected from atmospheric moisture by coating with paraffin or similar means. Such powders 45 also have a longitudinal center hole, for facilitating ignition and combustion.

The use of such packaged powder in stick form 50 brings many apparent advantages, not only in ease of handling and freedom from fire and explosion hazards, but in increased convenience in the loading of bore holes as well. In actual blasting, the powder may be used in whole packages or sticks having the length of approximately 8", or in portions of such sticks.

55 The object of my invention is to produce a

new and improved blasting powder in stick form, characterized by its high strength, this strength being capable of control by adjustment of the composition of the powder. A further object is a formed block of black blasting powder having 5 a relatively low density. Additional objects will be apparent as the invention is further described and disclosed hereinafter.

These objects are accomplished by including among other things ammonium nitrate as an ingredient in my improved powder. In such a composition, the ammonium nitrate replaces with beneficial results a portion of the sodium nitrate or other inorganic nitrates commonly used in such blasting powder compositions. I find, however, that it is not desirable to replace all the sodium nitrate in the powder by ammonium nitrate, since with such high percentages of ammonium nitrate, the powder tends to become a detonating rather than a deflagrating explosive. 20

I find that the replacement of a portion of the sodium nitrate by ammonium nitrate in black blasting powder compositions brings about increased explosive strength. This increase in strength is due principally to the fact that the 25 ammonium nitrate on combustion produces gaseous decomposition products only, whereas a considerable portion of the decomposition products of sodium nitrate is made up of solid materials. The increased strength of the ammonium nitrate powders results therefore from the increased gas volume from a given weight of powder. By replacing greater or smaller portions of the sodium nitrate heretofore used by ammonium nitrate, the strength of the powder may 30 be effectively controlled. I preferably use between 5 and 30% ammonium nitrate in my improved powder compositions, since less than 5% does not give the desired improved properties, while more than 30% ammonium nitrate renders 35 the powder less readily combustible and more subject to detonation.

The pelleted powders produced previously have had a greater strength than was necessary or desirable in many cases. For this reason, low 45 density powders have a very practical application, since by their use a smaller weight of explosive is required and a better distribution of the explosive pressure within the bore-hole is possible.

The incorporation of ammonium nitrate in black blasting powders in place of a portion of the sodium nitrate brings about a lower density in the finished explosive, due doubtless to the fact that the density of ammonium nitrate itself 50

is lower than that of sodium nitrate, approximately 1.72 against 2.27. I have found, however, that powders containing ammonium nitrate may be produced having much lower densities than 5 have been obtained heretofore. I obtain this result preferably by lightly packing the wet powder, having a water content between 4 and 8% for example, in a container which will preserve the form of the packed explosive and in which it 10 is dried and permitted to set into a hard block. The removal of the water from the powder brings about a relatively low density, which may be controlled by varying the pressure exerted in packing the powder into the shells.

15 While low density black blasting powder containing ammonium nitrate may be obtained in stick form, as described heretofore, I find that these low densities may readily be obtained by the introduction of low density carbonaceous 20 materials. While many different ingredients of this nature may be used, such as wood pulp, low density ingredients such as various vegetable piths, bagasse pith, cornstalk pith, and the like, I preferably use wood pulp because of its ready 25 availability and its satisfactory properties for such use. Fibrous carbonaceous material has the advantage of imparting cohesiveness as well as low density properties to the block of blasting powder.

30 I am aware that ammonium nitrate has been used as an ingredient of deflagrating blasting powders in the prior art. The use of ammonium nitrate, however, has particular advantage in the case of low density blasting powders. When incorporated into the formulas of high density 35 powders, ammonium nitrate retards the rate of combustion of the powder too greatly. I have found, however, that ammonium nitrate does not have this retarding effect in the low density powders according to my invention. At the same 40 time, the use of ammonium nitrate makes possible the maintenance of the bulk strength of the powder, even with greatly decreased densities and increased stick counts.

45 My invention therefore makes possible a new type of black blasting powder with desirable properties such as have been unattainable previously, namely the combination of high strength, low density, and satisfactory velocity of combustion.

50 By way of illustration of my invention by specific embodiments, the following examples are given of powder compositions showing the desirable properties imparted by the incorporation of 55 ammonium nitrate as an ingredient of black blasting powders in low density stick form.

the shells with one end of the shell open. When dry, the shells were closed and given a waterproof coating.

The summary table following, based on the foregoing tabulation, very clearly shows the effects of increasing ammonium nitrate contents and of decreasing densities with powders containing 10% ammonium nitrate, for example. It is seen that, as the density of the powder decreases, the rate of pressure development increases with 10 the strength remaining substantially constant for a given volume of powder, in spite of the lower weight. The same tendency is indicated with powders having the 20% content of ammonium nitrate. It will be seen, also, from the tabulation that an increase in the amount of ammonium nitrate present for a given density results in an increased rate of burning contrary to what would have been expected from experience with 15 high density powders.

5

10

15

20

25

| Ammonium nitrate | Density | No. of ctgs. per 50 lbs. | Bulk strength          |     | Velocity rate of press. devel. per ctg. |
|------------------|---------|--------------------------|------------------------|-----|-----------------------------------------|
|                  |         |                          | Max. pressure per ctg. | 25  |                                         |
| 0%.....          | 1.30    | 130                      | 30.7                   | 129 |                                         |
| 10.....          | 1.25    | 135                      | 29.9                   | 110 |                                         |
| 10.....          | 1.22    | 138                      | 28.9                   | 125 |                                         |
| 10.....          | 1.15    | 145                      | 30.8                   | 235 | 30                                      |
| 20.....          | 1.25    | 135                      | 34.5                   | 130 |                                         |
| 20.....          | 1.12    | 148                      | 33.4                   | 220 |                                         |
| 20.....          | 1.01    | 162                      | 31.4                   | 230 |                                         |

The examples cited in the tables heretofore have all been powders made from wheel cake, in order that the values obtained might be comparable. It should be understood, however, that my invention is intended to cover also blocks of powder made of grained powder, in which case higher rates of pressure development will be obtained.

35

40

50

By the use of ammonium nitrate as an ingredient, together with a fibrous carbonaceous material, it is possible to obtain powders of densities lower than 1.30 and weighing less than 175 grams 45 for a 1 1/4" x 8" cartridge, corresponding to not less than approximately 130 such cartridges to a 50-pound case. The lowest density shown in the table for such a powder is 1.01, and densities as low as 0.90 are attainable.

55

The strength values given in the tabulation are those obtained when a 1 1/4" x 8" cartridge of the powder is shot in a closed bomb of 20-liters volume, for example in the Bichel bomb. The values for the rate of pressure development were obtained also by the use of the same apparatus.

55

|    | Compositions                                               |      |      |      |      |      |      |      |
|----|------------------------------------------------------------|------|------|------|------|------|------|------|
|    | 1                                                          | 2    | 3    | 4    | 5    | 6    | 7    | 8    |
| 60 | Ammonium nitrate.....                                      | 0.0  | 0.0  | 10.0 | 10.0 | 10.0 | 20.0 | 20.0 |
|    | Sodium nitrate.....                                        | 72.0 | 70.5 | 60.5 | 60.5 | 60.5 | 50.5 | 50.5 |
|    | Charcoal.....                                              | 18.0 | 15.6 | 15.6 | 15.6 | 15.6 | 15.6 | 15.6 |
|    | Sulfur.....                                                | 10.0 | 8.6  | 8.6  | 8.6  | 8.6  | 8.6  | 8.6  |
|    | Calcium carbonate.....                                     | 0.0  | 1.3  | 1.3  | 1.3  | 1.3  | 1.3  | 1.3  |
|    | Wood pulp.....                                             | 0.0  | 4.0  | 4.0  | 4.0  | 4.0  | 4.0  | 4.0  |
|    | Apparent density.....                                      | 1.30 | 1.18 | 1.25 | 1.22 | 1.15 | 1.25 | 1.12 |
|    | Rate of press. dev. kg./sq. cm./sec./ctg.....              | 129  | 110  | 110  | 125  | 235  | 130  | 220  |
|    | Strength—Pressure dev. kg./sq. cm./ctg. (1 1/4" x 8")..... | 30.7 | 29.2 | 29.9 | 28.9 | 30.8 | 34.5 | 33.4 |
|    | Wt. ctg.—gms.—1 1/4" x 8".....                             | 178  | 163  | 168  | 164  | 156  | 168  | 153  |
|    | Ctg./50 lb. case.....                                      | 128  | 139  | 135  | 138  | 145  | 135  | 148  |

60

65

70 In the foregoing table, the powders shown were prepared by punching into 1 1/4" x 8" formed paper shells wet compositions of wheel cake powder having a moisture content between 6 and 7%. At this moisture content, the powder was soft 75 and cohesive. The powders were then dried in

It will be understood that many variations from the compositions cited may be made without departing from the spirit of the invention. The sodium nitrate, for example, may be replaced, if desired, by potassium nitrate, calcium nitrate, or other suitable inorganic nitrate. Ad- 70 75

ditions of suitable acid-accepting materials such as calcium carbonate may be made also, along with wood pulp or other fibrous carbonaceous material. I intend to be limited in my invention only as indicated by the following patent claims.

I claim:

1. A formed block of deflagrating blasting powder, characterized by its high strength and having a density less than 1.30, said block comprising a modified black powder composition containing ammonium nitrate as an ingredient.
2. A formed block of deflagrating blasting powder, characterized by its high strength and having a density between about 0.90 and less than 1.30, said block comprising a modified black powder composition containing ammonium nitrate as an ingredient.
3. A formed block of deflagrating blasting powder characterized by its high strength and having a density less than 1.30, said block comprising a modified black powder composition containing 5 to 30% ammonium nitrate.
4. A formed block of deflagrating blasting powder, characterized by its high strength and having a density between about 0.90 and less than 1.30, said block comprising a modified black powder composition containing 40 to 75% sodium nitrate, 1 to 20% charcoal, 1 to 20% sulfur, and 5 to 30% ammonium nitrate.
5. A formed block of deflagrating blasting powder, characterized by its high strength and low density of less than 1.30, comprising a modified black powder composition containing as in-

gredients ammonium nitrate and a low density carbonaceous material.

6. A formed block of deflagrating blasting powder, characterized by its high strength and low density of less than 1.30, comprising a modified black powder composition containing as ingredients ammonium nitrate and wood pulp.

7. A formed block of deflagrating blasting powder, characterized by its high strength and low density of less than 1.30, comprising a modified black powder composition containing 5 to 30% of ammonium nitrate and a low density carbonaceous combustible material.

8. A formed block of deflagrating blasting powder, characterized by its high strength and having a density between about 0.90 and less than 1.30, said block comprising a modified black powder composition containing as ingredients ammonium nitrate and wood pulp.

9. A formed block of deflagrating blasting powder, characterized by its high strength and having a density less than 1.30, said block comprising a modified black powder composition containing 5 to 30% ammonium nitrate and 1 to 10% of a low density carbonaceous combustible material.

10. A formed block of deflagrating blasting powder characterized by its high strength and having a density between about 0.9 and less than 1.30, said block comprising a modified black powder composition containing 5 to 30% ammonium nitrate, 40 to 75% sodium nitrate, 1 to 20% charcoal, 1 to 20% sulfur, and 1 to 10% wood pulp.

WILLIAM E. KIRST.